

## [54] FUEL COMPOSITION

[75] Inventors: Raymond Cadorette; George W. Eckert, both of Wappingers Falls, N.Y.

[73] Assignee: Texaco Inc., New York, N.Y.

[22] Filed: April 27, 1971

[21] Appl. No.: 137,981

[52] U.S. Cl. .... 44/72

[51] Int. Cl. .... C10I 1/22

[58] Field of Search .... 44/72; 424/325

## [56] References Cited

## UNITED STATES PATENTS

2,975,042 3/1961 Summers, Jr. .... 44/72  
2,975,043 3/1961 Ambrose .... 44/72  
2,246,524 6/1941 Kyrides .... 424/325

2,891,850 6/1959 Cosgrove et al. .... 44/72

Primary Examiner—Daniel E. Wyman

Assistant Examiner—Mrs. Y. H. Smith

Attorney—Thomas H. Whaley and Carl G. Ries

## [57] ABSTRACT

Hydrocarbon fuel composition in the gasoline and kerosene boiling ranges having bactericidal properties containing from about 0.001 to 0.005 weight percent of an N-alkyl-substituted-1,3-propanediamine having the formula:



in which R is an alkyl radical having from one to four carbon atoms and R' is hydrogen or an alkyl radical having from one to four carbon atoms.

7 Claims, No Drawings

## FUEL COMPOSITION

## BACKGROUND OF THE INVENTION

## 1. Field of the Invention

For many years, tetraalkyl lead compounds have been employed in gasoline to improve the octane quality of the fuel composition. The tetraalkyl lead compounds imparted a variety of valuable properties to gasoline in addition to improving the octane value. One of these properties was to inhibit the growth of bacteria in the gasoline composition. Bacteria are generally present in storage tank water bottoms and can grow rapidly in a light hydrocarbon fuel in the absence of an effective biocide or growth inhibitor.

Currently, anti-pollution drives and legislative thrust is being directed to the removal of tetraalkyl lead compounds from motor fuel composition. Unleaded gasolines are presently being marketed in response to these pressures. It has been observed, however, that one of the problems associated with some unleaded gasolines is that bacterial growth proceeds uninhibited in the fuel composition. This growth can proceed to the point where the bacteria formed cause fuel filter plugging in the fuel supply system of an engine.

## 2. Description of the Prior Art

U.S. Pat. No. 2,333,294 discloses a motor fuel composition having improved stability with respect to the formation of color and gum containing an alkylphenol in combination with a substituted alkylene diamine having the formula:



in which R is an alkyl group, R' and R'' may be an alkyl group or a hydrogen atom; wherein R''' may be a hydrogen atom, an alkyl group or an aminoalkyl group; y may be zero or an integer and y' is an integer. Representative compounds are N,N-diethyl ethylene diamine and N,N-di-n-butyl-ethylene diamine.

U.S. Pat. No. 2,891,850 discloses a motor fuel composition having improved carburetor anti-stalling properties containing an N-alkyl substituted diamine represented by the formula:



in which R<sub>1</sub> is an alkyl group containing from 10 to 30 carbon atoms; R<sub>2</sub>, R<sub>4</sub> and R<sub>5</sub> are hydrogen atoms or alkyl groups, at least two of which are hydrogen atoms; and R<sub>3</sub> is an alkylene group containing from two to six carbon atoms.

U.S. Pat. No. 2,961,309 discloses an anti-icing gasoline composition containing a minor amount of a glycol in combination with a mono-N-alkyl substituted-1,3-propanediamine wherein the alkyl group contains an average of 12 to 14 carbon atoms.

U.S. Pat. No. 2,987,385 discloses an anti-stalling gasoline composition containing the reaction mixture of lecithin and an N-aliphatic hydrocarbon substituted trimethylene diamine having the formula:



wherein R is an aliphatic hydrocarbon radical having from eight to 20 carbon atoms.

## SUMMARY OF THE INVENTION

The light distillate hydrocarbon fuel composition of the invention comprises a major portion of the mixture of hydrocarbons in gasoline and/or kerosene boiling ranges containing a minor bactericidal amount of N-alkyl-1,3-propanediamine having the formula:



in which R is an alkyl radical having from one to four carbon atoms and R' is hydrogen or an alkyl radical having from one to four carbon atoms.

More specifically, the fuel composition of the invention will comprise a mixture of hydrocarbons boiling in the range from about 70° to 625°F and will contain from about 0.001 to 0.005 weight percent of the prescribed bactericidal N-alkyl-substituted-1,3-propanediamine.

The discovery that a particular class of N-alkyl-substituted alkylene diamines is effective as a bactericidal additive when employed at a low concentration in a hydrocarbon fuel composition was unexpected. Tests on closely related compounds including N-alkyl-substituted-alkylene diamines and propanediamine showed that they had essentially no bactericidal properties when employed in light distillate hydrocarbon fuels in a low concentration.

Examples of the effective bactericidal N-alkyl-1,3-propanediamines within the scope of this invention include N-isopropyl-1,3-propanediamine, N,N-dimethyl-1,3-propanediamine, N-ethyl-1,3-propanediamine, N,N-diethyl-1,3-propanediamine and N-methyl-1,3-propanediamine.

The hydrocarbon fuel composition of the invention consists of any light distillate hydrocarbon fraction boiling in the gasoline and/or kerosene boiling ranges. The base fuel may consist of paraffinic, naphthenic and/or aromatic hydrocarbons or mixtures thereof suitable for use in either a spark-ignited or a turbine internal combustion engine. The base fuels are obtained from the distillation of crude oil, by the catalytic or thermal cracking of gas oils, by the alkylation of isoparaffins with olefins, or by the polymerization of olefins. The boiling range of the base fuel will generally be in the range from 70° to 625°F. Motor fuel or gasoline generally boils from about 90° to 425°F and kerosene base or turbine fuels generally boils from about 325° to 625°F. The base fuel composition may also contain additives conventionally employed in gasoline or kerosene, such as anti-oxidants, stabilizers, dyes, anti-icing additives and the like.

The fuel compositions of the invention were tested for their bactericidal property according to the following procedure: a sample of water was inoculated with a portion of a blood agar microorganism culture of typical microorganisms obtained from the water bottoms of a mineral fuel oil storage tank. Five cc of the inoculated water was covered with 20 cc of the fuel sample to be tested in a one ounce bottle. The stoppered bottle was maintained at room temperature for 5 days with daily agitation. At the end of this time approximately one drop of the water phase was placed on a blood agar plate which was then maintained at room temperature for 5 days or until a growth occurred, whichever came

first. A control fuel sample was run concurrently with the test fuels containing a biocide. The base fuel designated Base Fuel A employed in the following test was a premium grade unleaded gasoline boiling in the range from about 90° to 400°F. This fuel had a research octane number of about 91. This fuel consists of about 12 percent olefinic hydrocarbons, 25 percent aromatic hydrocarbons and 63 percent saturated hydrocarbons.

The test results are set forth in the table below:

|    |                                                  |       |                |
|----|--------------------------------------------------|-------|----------------|
|    | 1,3-propanediamine                               | 0.005 | no growth      |
| 3  | 3. Base Fuel B + N,N-dimethyl-1,3-propanediamine | 0.005 | no growth      |
| 5  | 4. Base Fuel B + N-oleyl-1,3-propanediamine      | 0.005 | profuse growth |
| 10 | Base Fuel B + N-tallow-1,3-propanediamine        | 0.010 | profuse growth |
| 15 | 6. Base Fuel B + propane-diamine                 | 0.005 | profuse growth |

TABLE I  
CULTURE TEST

| Fuel Composition                               | Additive Concentration | Culture Test Result |    |
|------------------------------------------------|------------------------|---------------------|----|
| 1. Base Fuel A                                 | none                   | profuse growth      |    |
| 2. Base + N-isopropyl-1,3-propanediamine       | 0.004                  | no growth           | 20 |
| 3. Base Fuel + N,N-dimethyl-1,3-propanediamine | 0.004                  | no growth           |    |
| 4. Base Fuel + N,N-diethyl-ethylenediamine     | 0.01                   | profuse growth      |    |
| 5. Base Fuel + N-coco-1,3-propanediamine       | 0.004                  | profuse growth      |    |

The base fuel employed in the following test was a mixture of straight run gasoline and straight run kerosene having the following values:

INSPECTION TEST ON BASE FUEL B (AVJET B)

|                              |           |
|------------------------------|-----------|
| Gravity, °API                | 56.7      |
| Distillation Temperature, °F |           |
| IBP                          | 75        |
| EP                           | 500       |
| Sulphur, %                   | 0.023     |
| Freezing Point, °F           | -76       |
| Heat of Combustion B.T.U./lb | ca 18,000 |
| Luminometer No.              | 50 to 55  |
| Aromatic Content, %          | 16 to 18  |

Fuel compositions according to the invention were tested for their bactericidal property in the manner described above as set forth in the following table.

TABLE II

RESULTS OF CULTURE TEST

| Fuel Composition             | Additive Concentration | Culture Test Result |  |
|------------------------------|------------------------|---------------------|--|
| 1. Base Fuel B               | none                   | profuse growth      |  |
| 2. Base Fuel B + N-isopropyl |                        |                     |  |

The foregoing data show that the fuel composition of the invention containing a prescribed N-alkyl-substituted 1,3-propanediamine had effective bactericidal properties. In contrast, related N-alkyldiamines had no bactericidal properties.

We claim:

1. A fuel composition comprising a mixture of hydrocarbons boiling in the range from about 70° to 625°F containing from about 0.001 to 0.005 volume percent of an N-alkyl-substituted-1,3-propanediamine having the formula:



25 in which R is an alkyl radical having from one to four carbon atoms and R' is hydrogen or an alkyl radical having from one to four carbon atoms.

3. A fuel composition according to claim 1 in which said N-alkyl-substituted-1,3-propanediamine is N-isopropyl-1,3-propanediamine.

3. A fuel composition according to claim 1 in which N-alkyl-substituted-1,3-propanediamine is N,N-dimethyl-1,3-propanediamine.

4. A fuel composition according to claim 1 in which 35 said N-alkyl-substituted-1,3-propanediamine is N-ethyl-1,3-propanediamine.

5. A motor fuel composition according to claim 1 boiling in the range from about 90° to 425°F.

6. A turbine fuel composition according to Claim 1 40 boiling in the range from about 325° to 625°F.

7. A method for producing a light hydrocarbon fuel composition having bactericidal properties which comprises adding from about 0.001 to 0.005 volume percent of an N-alkyl-substituted-1,3-propanediamine to a 45 light distillate hydrocarbon fuel composition boiling in the range from about 70° to 625°F, said N-alkyl-substituted-1,3-propanediamine having the formula:

50  $H_2N-CH_2CH_2CH_2NRR'$  in which R is an alkyl radical having from one to four carbon atoms and R' is hydrogen or an alkyl radical having from one to four carbon atoms.

\* \* \* \* \*